

## UNITED STATES PATENT OFFICE

2,365,402

## TEXTILE PROCESS AND PRODUCT

Robert N. Foster, Anniston, Ala., assignor to  
Monsanto Chemical Company, a corporation of  
Delaware

No Drawing. Application November 28, 1940,  
Serial No. 367,575

19 Claims. (Cl. 28—72.6)

This invention relates to an improved textile size and products produced therewith.

An object of this invention is the provision of a new sizing agent of an inorganic nature which may be readily applied to textile fibers and which may be easily removed therefrom by merely washing with water.

My new size may be applied to fibers of cotton, linen, flax, hemp, jute, ramie, the various rayons, staple or filament such as viscose, acetate and cuprammonium or the various synthetic polymeric organic compounds used as textile fibers as nylon, vinyon, etc., including glass textile fibers.

Used as a size my product is effective upon the yarns of the above mentioned fibers and others, for the purpose of laying the fiber ends, setting the twist and providing a coating to resist mechanical wear, and increase strength particularly for the warp yarns used in weaving.

My sizing compound is a phosphate of colloidal nature and is composed of the metaphosphates of potassium and sodium having the general formula  $K_mNa_{(6-m)}(PO_3)_6$  where  $m$  may have a value of 2 or less, including fractional values. There may also be present mixtures of the above.

One of the phosphates of the above type has been described by Tammann in Zeit fur prakt. chem. 45, 417 (1892). The Tammann phosphate has the composition,  $K_2Na_4(PO_3)_6$ , and was called by him dipotassium tetrasodium hexametaphosphate.

While there may be some doubt about the state of molecular aggregation of these phosphates that is whether they are hexa metaphosphates or of some other degree of molecular aggregation they are known to embody the stoichiometric composition expressed by the formulae given above.

Accordingly, from this standpoint, the mixed phosphates of potassium and sodium usable in my process comprise a series varying in composition as indicated by the formula:



where  $m$  may have a value of 2 or less, including fractional values. An analysis of two members of this series will show the following chemical composition:

|          | Theory for<br>$K_2Na_4(PO_3)_6$ | Theory for<br>$K_1Na_5(PO_3)_6$ |
|----------|---------------------------------|---------------------------------|
| $K_2O$   | 14.62                           | 7.50                            |
| $Na_2O$  | 19.25                           | 24.67                           |
| $P_2O_5$ | 63.13                           | 67.83                           |

Phosphates of this series have the property of forming viscous aqueous solutions of a colloidal nature, the viscosity of which may be varied by changing the concentration. Apparently the colloidal particles are strongly hydrated. As an example of the viscosity and specific gravity of aqueous solutions of these phosphates, I give the following data for the  $K_2Na_4(PO_3)_6$  compound at 30° C.

|                          | Concentration |      |       |       |       |      |
|--------------------------|---------------|------|-------|-------|-------|------|
|                          | 1%            | 5%   | 10%   | 15%   | 20%   | 30%  |
| 15 Specific gravity..... | 1.005         | 1.04 | 1.075 | 1.125 | 1.175 | 1.25 |
| Viscosity.....poises     | 0.09          | 0.36 | 0.76  | 2.1   | 6.9   | 178  |

The colloidal phosphate solutions herein employed may be prepared by the reaction of  $KPO_3$  with sodium chloride solution (the method described by Tammann) or by the direct reaction of  $KPO_3$  and  $(NaPO_3)_6$  according to the reaction:



25 In the application of these phosphates for the sizing of textile fibers I prefer to make a 15% solution of the phosphate and wet the yarn in this solution. After removing the fiber from the solution, it is dried and the phosphate then forms 30 a transparent flexible non-tacky film upon the fiber; this lays the fiber ends, sets the twist and provides an abrasion resistant protective coating. The coated, dried yarn, may hold from 15 to 20% by weight of phosphate, however the amount of 35 phosphate carried by the yarn may be varied over a wide range. In general from 1% to more than 30% by weight of phosphate may thus be applied.

40 My size may be applied by means of a "slasher" as currently used in the silk or cotton textile mill practice. In these machines substantially the above process is carried out, and drying is effected either by means of heated rolls or by a current of warm air.

45 The sizing bath employing my phosphates may be heated somewhat although in contrast with the customary starch sizing baths it is not necessary or desirable to heat the bath to the boiling point. My size is preferably applied cold, that is at room temperature to a temperature of 50 or 55° C. under which conditions good penetration is obtained upon viscose rayon, cuprammonium rayon, degummed flax or bleached cotton. Using raw cotton or the non-absorbent fibers such as acetate rayon, nylon or vinyon it is 50 preferable to employ a wetting agent in the sizing

bath. While any type of wetting agent which will give good penetration may be employed, I have used with good results agents of the sodium alkyl aryl sulfonates, the alkyl chain having from 8 to 16 carbon atoms in the molecule. The amount of wetting agent employed may be from 0.01% to 1 or more percent based upon the weight of the bath.

The tensile strength of ordinary unscoured, unbleached cotton yarn treated with my size is approximately twice that obtained with a regular starch size, without material sacrifice of elasticity.

A great advantage of my size is that the size can be easily removed from the fibers by simple extraction using either cold or warm water. Starch sizes on the other hand require more drastic treatments, for example, treatment with acids, alkalies or enzymes to remove the starch.

While my phosphate size may be employed by itself and good results obtained, for special purposes I may add softeners or preservatives for mildew prevention as is customary when applying commercial starch sizes.

Examples of softeners used with my size are sulfonated oils such as castor or olive oils or sulfonated waxes such as tallow, etc.

Preservatives suitable for mildew prevention may be zinc chloride, pentachlorophenols, o-hydroxydiphenyls, etc.

If the production of sized goods is contemplated, the size need not necessarily be removed after weaving, in fact woven goods may be filled or sized using the colloidal phosphate size. If the goods are to be kier boiled, the phosphate will dissolve out from the fiber and furthermore serves the purpose of a water-softener combining with the calcium and magnesium hardness of processing water and rendering them harmless or innocuous during processing. During kiering it will also serve to prevent kier stains on the cloth as from iron, etc. The phosphate size is also advantageously utilized in bleaching or in dyeing as the deleterious effects of hard water causing stains or uneven dyeing are thereby eliminated, by virtue of a combination of the sizing phosphates with the calcium and magnesium hardness, usually present in the water.

Paper sizes comprising casein and hexametaphosphates of sodium or other alkali metals have been proposed, however in these earlier proposals, the hexametaphosphate served as a solubilizing compound or emulsifying agent for the casein. In my invention the double metaphosphates of sodium and potassium, that is where both sodium and potassium are contained in a single molecule of the metaphosphate, are employed per se as sizing agents.

What I claim is:

1. A method of processing textile warp yarns comprising treating said yarns with a colloidal solution of a phosphate of the composition:  $K_mNa_{(6-m)}(PO_3)_6$  in which  $m$  has a value of from 2 to 1, to apply a size thereon, weaving said yarn on a loom to produce woven goods, treating said goods subsequently with water containing calcium and magnesium hardness, whereby said calcium and magnesium hardness is rendered innocuous by reaction with said size, and the size simultaneously removed from said warp yarn.

2. The process defined in claim 1 in which the colloidal phosphate employed as a size is a compound selected from the class consisting of  $K_2Na_4(PO_3)_6$  and  $K_1Na_5(PO_3)_6$ .

3. The process defined in claim 1 in which the colloidal phosphate employed comprises a mix-

ture of the compounds  $K_2Na_4(PO_3)_6$  and  $K_1Na_5(PO_3)_6$ .

4. A method of processing cotton yarn comprising applying to said yarn a size comprising a colloidal phosphate of the composition  $K_mNa_{(6-m)}(PO_3)_6$  in which  $m$  has a value of from 2 to 1, weaving said yarn upon a loom to produce woven goods, subsequently processing said woven goods by kiering with a water solution carrying calcium and magnesium hardness, whereby said size is removed from the goods and is combined with said calcium and magnesium hardness to soften said processing water.

5. A method of processing rayon yarn comprising applying to said yarn a size comprising a colloidal phosphate of the composition  $K_mNa_{(6-m)}(PO_3)_6$  in which  $m$  has a value of from 2 to 1, weaving said yarn upon a loom to produce woven goods, thereupon dyeing said woven goods in a water solution containing calcium and magnesium hardness, whereby said size is removed by said dye bath and combined with said calcium and magnesium hardness, preventing combination thereof with said dye.

6. A textile yarn suitable for warp threads comprising spun fibers carrying a transparent flexible, water soluble film of Tammann's dipotassium tetrasodium hexametaphosphate.

7. A textile yarn suitable for use as a warp thread in weaving comprising spun fibers carrying a transparent, flexible, water soluble film of the salt:  $K_mNa_{(6-m)}(PO_3)_6$  in which  $m$  has a value of from 2 to 1.

8. A process of treating fiber for the production of a size thereon, comprising wetting said fiber with a colloidal solution of a compound selected from the class consisting of  $K_2Na_4(PO_3)_6$  and  $K_1Na_5(PO_3)_6$ .

9. A method of treating textile warp yarns comprising sizing said yarns with a colloidal solution of a phosphate of the composition:  $K_mNa_{(6-m)}(PO_3)_6$ , in which  $m$  has a value varying from a positive fractional value to a value of 2 and weaving said yarn upon a loom to produce woven goods.

10. The method defined in claim 9 wherein a 15% solution of the phosphate is employed in sizing the yarns.

11. The method defined in claim 9 wherein the woven goods are subsequently treated with water containing calcium and magnesium hardness, whereby said calcium and magnesium hardness is rendered innocuous by reaction with said size, and the size is simultaneously removed from said warp yarn.

12. A method of processing textile warp yarns comprising sizing said yarns with a colloidal solution of mixed phosphates of potassium and sodium varying in composition according to the formula:  $K_mNa_{(6-m)}(PO_3)_6$ , where  $m$  represents a value varying from a positive fractional value to a value of 2.

13. The method defined in claim 12 in which  $m$  represents a value of from 2 to 1.

14. A method of processing textile fibers comprising sizing said fibers with a colloidal solution of a phosphate having a stoichiometric composition expressed by the formula:  $K_mNa_{(6-m)}(PO_3)_6$ , in which  $m$  has a value of 2 to 1 and drying the product thus formed.

15. A method of sizing textile fibers comprising immersing said fibers in a bath containing a colloidal solution of a phosphate having a stoichiometric composition expressed by the formula:

$K_mNa_{(6-m)}(PO_3)_6$ , in which  $m$  has a value of 2 to 1.

16. The method defined in claim 15 wherein the bath contains a wetting agent.

17. The method defined in claim 15 wherein the bath contains 0.01 to 1% by weight of a wetting agent.

18. The method defined in claim 15 wherein

the bath contains as a wetting agent, a sodium salt of an alkylated aromatic sulfonic acid having from 8 to 16 carbon atoms in the alkyl chain.

19. A textile fiber carrying a transparent flexible film of a phosphate having a stoichiometric composition expressed by the formula:  $K_mNa_{(6-m)}(PO_3)_6$ , in which  $m$  has a value of 2 to 1.

ROBERT N. FOSTER.